

Feb. 10, 1948.

R. FRANKS

2,435,624

WEATHER RESISTANT STEEL AND ARTICLES

Filed June 3, 1944

(A)



3% CR; 0.06% C.  
BHN = 131

(B)



NO CR; 0.09% C.  
BHN = 107

*Fig. 1.*

(A)



3% CR; 0.16% C.  
BHN = 293

(B)



4.5% CR; 0.07% C.  
BHN = 311

*Fig. 2.*

(A)



3% CR; 0.06% C.  
BHN = 128

(B)



NO CR; 0.09% C.  
BHN = 107

*Fig. 3.*

INVENTOR  
RUSSELL FRANKS

BY

*Ernest Greenwald*  
ATTORNEY

## UNITED STATES PATENT OFFICE

2,435,624

## WEATHER RESISTANT STEEL AND ARTICLES

Russell Franks, Niagara Falls, N. Y., assignor to  
Electro Metallurgical Company, a corporation  
of West Virginia

Application June 3, 1944, Serial No. 538,615

8 Claims. (Cl. 75—126)

1

This invention relates to weather-resistant steel and to articles in the form of sheets, strips or wire fabricated from such steel and suited for use, for instance, as roofing, siding, gutters, drain pipes, smoke stacks, and fencing, for buildings, boats, and other structures exposed to the weather. The invention also relates to steel having good impact strength at subzero temperatures and to articles fabricated from such steel suitable for use under conditions wherein they are subjected to impact shock or multi-dimensional stress at subnormal temperatures. This latter class of articles includes, for instance, pressure vessels and machine elements used at high altitudes or in arctic regions or in refrigerating apparatus.

The principal object of the invention is to provide a mild steel and articles made therefrom characterized by resistance to progressive rusting, by good properties of strength, ductility and toughness, by retention of toughness at subzero temperatures and by ease of fabrication by rolling, bending, drawing, welding and other conventional methods.

It has been widely recognized for many years that the rusting of iron and steel structures results in a tremendous loss of wealth not only through the destruction of the structural steel itself but also through the expense involved in maintenance of such structures. Painting, resorted to as a means of inhibiting rusting, is an unsatisfactory expedient at best. Any break in a paint film on a painted carbon steel structure exposed to the weather becomes the center of a rapidly widening area of rusting. The rusting proceeds under the paint film and in time the latter falls away. Therefore, painting on a large structure is a never-ending task and expense.

Although there are available so-called stainless or rustless steels and irons, these materials owe the principal part of their very great resistance to corrosion to a substantial content of chromium, the chromium content being upwards of 10%. These highly alloyed steels are far too expensive to use for non-ornamental parts of large structures subject to corrosive conditions no more severe than ordinary weathering.

Steels containing about 4% to 6% chromium are widely used to resist mild corrosives. The steels are less expensive than the stainless or rustless steels, and their resistance to corrosion by mild corrosives is good. However, the engineering properties of these steels are such that they are ill suited to use in the fabrication of structures of the kinds under discussion. Addi-

tionally, these steels upon prolonged exposure to the weather are susceptible to the formation of surface pits, the effects of which to a degree offset the advantages of the resistance of the steels to generalized surface corrosion. A further disadvantage of the steels which renders their use for the fabrication of structures of the type under discussion commercially impractical is that their cost is very materially greater than that of ordinary structural steels.

Medium chromium steels containing about 3% chromium and more than 0.1% carbon have been investigated in the past. These steels have a metallographic structure profoundly different from that of plain carbon steels, and they are air hardening, that is harden on cooling in still air from temperatures above the upper critical point. Because of their air hardening characteristic they are not amenable to fabrication into articles of the kind under discussion by standard methods of hot working such as hot rolling or by welding since they can not be permitted to cool rapidly from the temperatures employed in such operations.

In recent years a number of low alloyed steels containing fractions of 1% of chromium and either copper or phosphorus have come into use for engineering and structural purposes. The principal advantage of these steels lies in their high strength. They are also appreciably more resistant to progressive rusting than the ordinary carbon structural steels, but their improved resistance to rusting alone would not justify the use of these steels for the fabrication of structures exposed to the weather.

The invention comprises steels, and articles made therefrom, containing between 2.75% and 3.5% chromium, 0.01% to 0.08% carbon, 0.1% to 0.6% silicon, 0.1% to 0.6% manganese, remainder iron and the incidental impurities commonly present in steels of good quality, which steels are resistant to deterioration on prolonged exposure to the weather, are readily workable by ordinary methods of fabrication, and are strong at low temperatures. The invention also includes a method of working such steels.

The accompanying drawing is based on photomicrographs taken at an original magnification of 250 diameters. In preparing the drawing, the photomicrographs were somewhat enlarged, and the lines in the drawing are somewhat exaggerated in thickness. In the drawing:

Figs. 1A and 1B are representations of the microstructure of a low carbon 3% chromium

steel and of a plain low carbon steel, respectively, in one condition of heat treatment;

Figs. 2A and 2B are representations of the microstructure of a 3% chromium steel containing more carbon than the steel of Fig. 1A and of a low carbon, 4.5% chromium steel, respectively, in the same condition of heat treatment; and

Figs. 3A and 3B are representations of the microstructure of the steels illustrated in Figs. 1A and 1B but in a different condition of heat treatment.

I have discovered in the course of tests running continuously for periods as long as ten years that the steels of the invention are strongly resistant to progressive rusting by weathering and have no tendency to form pits on prolonged exposure to the weather. Moreover, they behave metallurgically like mild plain carbon steel. They may be rolled in standard commercial mills into the standard structural shapes including sheets and strips, and may be drawn to wire or cut, welded, riveted and otherwise handled by the methods used in fabricating large structures from ordinary carbon steels. Further, these steels may be made in the open hearth furnace, one of the least expensive ways to make steel.

The resistance of these steels to weathering, even when unpainted, is remarkable. For instance, over a 10 year exposure of unpainted test samples to the weather in two successive industrial neighborhoods, a mild steel 20 gauge sheet containing 0.15% carbon, remainder iron and incidental impurities, lost an average of 0.11 gram per square inch per year and, in the ten years suffered a decrease in thickness averaging 49% and in places amounting to 62%; while a mild steel 20 gauge sheet containing 0.07% carbon, 3.05% chromium, remainder iron and incidental impurities, lost an average of but 0.023 gram per square inch per year, or about  $\frac{1}{5}$  of the average loss of the plain carbon steel, and suffered a decrease in thickness in ten years averaging over the sample only 8% and being at no point greater than 20%. The loss in weight of a similarly exposed test sample of steel containing 5.60% chromium and 0.07% carbon was at a rate of 0.021 grams per square inch per year, immaterially different from that of the 3% chromium steel, and this sample was deeply pitted.

These test results, as well as other similar results, clearly indicate that the low carbon 2.75% to 3.25% chromium steels of the invention are importantly more resistant to weathering than plain carbon steels and that raising the chromium content to about 6% imparts no material additional resistance to progressive rusting and may even be detrimental from the standpoint of resistance to weathering since steels containing about 4% to 6% chromium are susceptible to pitting on prolonged exposure to the weather.

The steels of the invention may be readily worked by the ordinary methods employed in working plain carbon steels and within the usual temperature ranges. Thus, no difficulty is encountered in working the steels at temperatures above or just below the critical range. No changes in ordinary working procedure are necessary to accommodate the steels of the invention.

One reason for the ready workability of the steels of the invention are their freedom from the air hardening tendencies usually associated

with medium chromium steels. Extensive tests have indicated that the percentage of chromium and the percentage of carbon present in the steels of the invention are critical. Steels containing no more than about 3.25% chromium and 0.08% carbon may be rapidly cooled in air from temperatures above the upper critical point without hardening. If however, the chromium content is raised only to about 4%, tests have shown that the steel will harden considerably on air cooling from above the upper critical point even though the carbon content is as low as 0.08%. Similarly, steel containing 0.1% carbon or more will harden on air cooling from temperatures above the upper critical point even if the chromium content is no more than 3.25%. Accordingly, to achieve one of the most important benefits of the invention, both the upper limit of chromium and the upper limit of carbon must be observed strictly.

In Figs. 1 and 2 of the drawing there are reproduced photomicrographs of a low carbon 3% chromium steel containing 0.06% carbon (Fig. 1A), a plain carbon steel (Fig. 1B) containing 0.09% carbon, a 3% chromium steel containing 0.16% carbon (Fig. 2A), and a low carbon 4.5% chromium steel containing 0.07% carbon (Fig. 2B), all of which steels are in the condition resulting from heating 10 minutes at 1650° F. followed by cooling in still air. In this condition the Brinell hardness ("BHN") of the low carbon 3% chromium steel is 131 and that of the plain low carbon steel is 107, while the Brinell hardness of the low carbon 4.5% chromium steel is 311 and that of the 3% chromium steel containing 0.16% carbon is 293. These values show that the hardness of the low carbon 3% chromium steel in this condition of heat treatment is only slightly greater than that of the plain low carbon steel but that an increase of chromium or carbon to proportions outside the ranges of those elements recited above results in pronounced air hardening.

The effect of chromium and carbon contents greater than 3.25% and 0.08% respectively on metallographic structure is evident from a comparison of the photomicrographs reproduced in Figs. 1 and 2 of the drawing. The structure of the low-carbon 3% chromium steel (Fig. 1A) is predominantly ferritic (light areas) with patches of a pearlitic constituent (dark areas). Comparison with the plain low carbon steel (Fig. 1B) shows that the structures of these two steels are very similar, the carbon steel also containing principally ferrite with some pearlite areas. However, in the case of the steel containing 3% chromium and 0.16% carbon (Fig. 2A) a very different structure is revealed. Here the structure is primarily pseudomartensitic containing a small amount of chromium ferrite (light areas), and is similar to that of the 4.5% chromium steel containing 0.07% carbon (Fig. 2B).

The ductility of the steels of the invention, as measured by elongation and reduction of area in tensile tests, is equal to or better than the ductility of plain carbon steels, and the yield strength and tensile strength of the steels of the invention are considerably higher than the yield strength and tensile strength of the ordinary carbon steels. For example, in the hot rolled condition the yield strength at 0.2% offset of an ordinary carbon steel containing 0.09% carbon is in the neighborhood of 47,000 pounds per square inch while the yield strength at 0.2%

offset of a hot rolled steel containing 0.06% carbon and 3.03% chromium is about 61,500 pounds per square inch. The tensile strength of the plain carbon steel is about 58,000 pounds per square inch, while the tensile strength of the 3% chromium steel is about 81,000 pounds per square inch. These values are typical of those measured in the direction of rolling.

For the best combination of ductility and toughness, the steels of the invention may be heat treated by heating them to a temperature just below the lower critical point, for example, between about 1250° F. and 1400° F., and cooling in air from this temperature. The effect of this subcritical heat treatment on the microstructure of the steels of the invention is illustrated in Fig. 3A of the drawing. In Fig. 3 there are reproduced photomicrographs of a 3% chromium steel containing 0.06% carbon (Fig. 3A) and of a plain carbon steel containing 0.09% carbon (Fig. 3B), both of which steels are in the condition resulting from heating 2 hours at 1340° F. and cooling in air. In both instances it is evident that the carbides present in the original pearlitic constituents of the steels have been spheroidized. By this heat treatment both the impact strength and the ductility of the steels of the invention are materially improved with only a slight decrease in the yield strength.

Ordinary carbon steels, even of very low carbon content, lose their shock resistance and become "notch brittle" at even moderately subnormal temperatures, for instance below -40° F. This is a matter of some concern, and has led to the use of nonferrous metals or special steels, usually austenitic steels, for many articles which otherwise would be made of carbon steel.

In strong contrast to plain carbon steel, the steels of the invention have good impact strength at subzero temperatures. Their retention of toughness is particularly notable after the subcritical heat treatment just described. For instance, a steel containing 3.07% chromium and 0.075% carbon had an impact strength at room temperature, after having been heated 2 hours at 1340° F. and air cooled, of 86 foot pounds as measured by the Izod impact test. Tests at 32° F., -40° F., -90° F., -150° F., and -190° F. indicate that the impact strength of this steel in this condition of heat treatment is substantially unchanged at temperatures at least as low as -190 F. Thus, the steel had an impact strength at -190° F. of 76 foot pounds, and at the other temperatures just recited had an impact strength of 81 to 83 foot pounds. Even in the condition resulting from cooling in air from a temperature above the upper critical point, the impact strength of the steel is in the neighborhood of about 20 foot pounds at -190° F. The impact strength of the same steel after having been heated above the upper critical point, air cooled, then reheated to just below the lower critical point and air cooled was of the same order as when the steel was merely given the subcritical heat treatment.

The steels of the invention may be welded by fusion-deposition methods using as filler metal rods of substantially the same composition. Tests have indicated that sound, strong welds are readily produced and that the welds retain their desirable properties at temperatures at least as low as -40° F.

The properties of the steels of the invention

are thus such as to make them eminently suitable for the fabrication of articles which are required to withstand exposure to the weather or of articles which are required to withstand impact or multi-dimensional stress at subzero temperatures. Because the steels can be made in the open hearth furnace and because they may be fabricated into structures by standard methods with standard equipment, the increase in cost of the steels when compared to ordinary carbon steel is reduced to a minimum, and their resistance to progressive rusting makes possible sufficient saving in maintenance expense to more than offset its additional cost.

I claim:

1. Weather-resistant mild steel substantially free from air hardenability, consisting substantially of chromium ferrite and chromium pearlite, and composed of 2.75% to 3.25% chromium, 0.01% to 0.08% carbon, 0.1% to 0.6% silicon, 0.1% to 0.6% manganese, remainder iron and incidental impurities.
2. Steel articles required to withstand corrosive attack on prolonged exposure to weather composed of the steel claimed in claim 1.
3. Steel as claimed in claim 1, in the condition produced by heating at a high temperature not far below the lower critical point and thereafter rapidly cooling.
4. Weather-resistant steel fencing composed of the steel claimed in claim 1.
5. Weather-resistant thin sheet metal roofing and siding composed of the steel claimed in claim 1.
6. Weather-resistant thin sheet steel containers composed of the steel claimed in claim 1.
7. Steel articles for use at subzero temperatures, which articles maintain an impact toughness of at least 20 foot pounds Izod at temperatures down to -200° F., composed of the steel claimed in claim 1.
8. Method of making weather-resistant mild steel sheet, strip, and wire which comprises hot working from above to just below the critical temperature a chromium ferrite-pearlite material composed of 2.75% to 3.25% chromium, 0.01% to 0.08% carbon, 0.1% to 0.6% silicon, 0.1% to 0.6% manganese, remainder iron and incidental impurities, such composition being characterized by freedom from air hardenability; heating the worked material to an elevated temperature not far below the critical temperature; and air cooling the so heated material.

RUSSELL FRANKS.

#### REFERENCES CITED

The following references are of record in the file of this patent:

#### UNITED STATES PATENTS

| Number    | Name        | Date           |
|-----------|-------------|----------------|
| 1,287,153 | Weitzenkorn | Dec. 10, 1918  |
| 1,110,395 | Lucertini   | Sept. 15, 1914 |
| 2,206,370 | Scherer     | July 2, 1940   |
| 2,315,156 | Larrabee    | Mar. 30, 1943  |

#### FOREIGN PATENTS

| Number  | Country | Date        |
|---------|---------|-------------|
| 797,842 | France  | May 5, 1936 |

#### OTHER REFERENCES

Bullens, Steel and Its Heat Treatment, vol 1, page 115.

**Certificate of Correction**

Patent No. 2,435,624.

February 10, 1948.

**RUSSELL FRANKS**

It is hereby certified that errors appear in the printed specification of the above numbered patent requiring correction as follows: Column 5, line 52, for "—190 F." read —190° F.; column 6, line 32, claim 5, for the word "metal" read *steel*; and that the said Letters Patent should be read with these corrections therein that the same may conform to the record of the case in the Patent Office.

Signed and sealed this 27th day of April, A. D. 1948.

[~~REDACTED~~]

**THOMAS F. MURPHY,**  
*Assistant Commissioner of Patents.*